

Nov. 9, 1937.

B. S. WHITE

2,098,268

METHOD OF MAKING SUBLIMED LITHARGE

Filed Sept. 26, 1934



INVENTOR  
**BERNARD S. WHITE**  
BY *Milton Jucker*  
ATTORNEY

## UNITED STATES PATENT OFFICE

2,098,268

## METHOD OF MAKING SUBLIMED LITHARGE

Bernard S. White, Hammond, Ind., assignor to  
The Glidden Company, Cleveland, Ohio, a corporation of Ohio

Application September 26, 1934, Serial No. 745,601

2 Claims. (Cl. 23—146)

This invention relates to lead oxide, and has particular reference to a new and novel method of preparing fumed lead oxide (sublimed litharge), whereby unusually high yields of the fumed product are obtained. More specifically, it contemplates feeding a partially oxidized lead oxide powder directly into a Bunsen flame, thus subjecting it to the extremely high temperatures of the flame, whereby the bulk of the crude 5 product is completely oxidized to lead monoxide, and is at the same time sublimed into the vapor phase.

Heretofore, the common practice in making sublimed litharge has been to blow a strong blast 15 of air over molten litharge, whereby the air current takes up the litharge vapor formed, or, alternately, to spray molten lead into a furnace, together with some fuel. Both methods are objectionable, in that the yield of the sublimed 20 product is low, and the resultant residue generally must be reworked to produce a marketable product.

It has also been proposed to blow a partially 25 oxidized lead oxide into a furnace, as set out in my applications, Serial Numbers 692,869 and 692,870. The resultant process is superior to those commonly practiced heretofore, in that considerably higher yields are obtained of fumed 30 product; and, if furnace conditions are kept right, the residue is marketable litharge. However, the yield of the fumed product leaves much to be desired. If a strong draft is maintained in the furnace, the yield is somewhat higher, but a considerable quantity of unsublimed ordinary 35 lead oxide is carried over to contaminate the fumed product. Higher yields may also be obtained by increasing furnace temperatures; but if the furnace is hotter than 1,325° F., the residue becomes pasty, and the resultant product 40 cannot be marketed without some after-treatment.

I have discovered that if a crude litharge is fed directly into a Bunsen type flame, the lead 45 oxide is very largely simultaneously oxidized and sublimed. A slight draft may be maintained up the flue, to keep the furnace gases moving; and the furnace should be kept at temperatures below 1,325° F., if it is desired to obtain directly a residue of marketable litharge. The yield of 50 sublimed litharge is very much higher than in the case of my old process, approaching 80% when furnace conditions are maintained properly; and the sublimed product is substantially free from ordinary litharge.

The details of my process may be most easily

understood by referring to the accompanying drawing, which is a conventionalized cross-section of the apparatus I prefer to employ, with the burner enlarged out of scale for clarity. A chamber (1) is provided, with furnace walls (2). Extending into one wall of the furnace is a burner (3) into which a gas pipe (4) and an air pipe (5) open. Crude litharge is placed in the hopper (6); it discharges into the mixed air and gas in the burner, being drawn into the burner partially 10 by suction and partially by gravity. The mixture of oxide, gas and air discharge through the nozzle (7) and burn in the Bunsen type flame (8). The fumed oxide is drawn through a flue (9) by the slight draft produced by a fan (10) 15 driven by a motor (11); it collects in a dust-collector (12). The oxide which is not sublimed, or which condenses in the furnace, collects as a pile (13) on the floor of the furnace, from whence it may be raked through a door (14) into containers, for use as ordinary litharge. 20

The raw material for the process may be any partially oxidized lead oxide. Crude "green" litharge, obtained by blowing air through pots of molten lead while keeping the lead agitated, is 25 a satisfactory starting product, as is lead suboxide. Powdered lead may be used in the process, but is not preferred, as unless extreme care is taken, the residue on the floor of the furnace may contain some unoxidized lead.

Furnace temperatures are likewise of considerable importance. The furnace temperatures must be maintained low enough so that the unsublimed residue will not sinter, so as to require milling; I preferably keep the temperature below 1,325° F., which is the point at which the residue becomes pasty. The flue temperature should, however, be high enough so that there will be no red lead in the sublimed oxide. For that reason, flue temperatures should preferably 30 be above the decomposition point of red lead; I prefer to operate at 1,050° F., just above that point.

The ratio of air to gas should of course be so regulated as to give complete oxidation of the 45 gas and crude raw material, without undue dilution of the gas stream. If it is not desired to obtain a directly marketable residue in the furnace, furnace temperatures may be increased to increase the yield. The pasty residue may then 50 be ground, and reworked; it is a satisfactory raw material for the process. In the event that the process is run in this manner, lead powder may, of course, be used as the raw material.

While the apparatus described shows the pre- 55

ferred form of my invention, other apparatus may be used without departing from the spirit of my invention, the essence of which lies in the simultaneous oxidation and sublimation by the 5 intense heat of a Bunsen flame.

In the claims, sublimed litharge is used to indicate the fumed product, litharge to indicate ordinary lead oxide, and lead-bearing powder to indicate the metal powder, or an oxidized lead 10 raw material.

I claim:  
1. The process of making litharge and sublimed litharge, which comprises mixing air, a combustible gas and lead oxide bearing powder 15 before ignition, burning the mixture in a furnace whose lower portion is maintained at or below 1,325° F., collecting litharge on the floor of the

furnace, drawing the sublimed litharge through a flue maintained at or above 1,050° F. and separating the sublimed litharge from the flue gases.

2. The method of fractionating a mixture of litharge vapor and litharge dust in a gas stream, comprising forming such a mixture by feeding oxidized lead into an oxidizing flame in a muffle furnace, allowing unvaporized dust to settle and collect in a portion of the combustion chamber adjacent the gas stream while maintaining that 10 portion of the furnace at or below 1,325° F. by regulation of the flame, and drawing the sublimed litharge through a flue maintained at or above 1,050° F., and separating the sublimed litharge from the flue gases. 15

BERNARD S. WHITE.